

# United States Patent [19]

Sakakura et al.

[11] 3,853,641

[45] Dec. 10, 1974

[54] **METHOD FOR PRODUCING  
SINGLE-ORIENTED SILICON STEEL  
SHEETS HAVING HIGH MAGNETIC  
INDUCTION**

[75] Inventors: Akira Sakakura; Satoru Taguchi; Toshiya Wada; Kiyoshi Ueno; Takaaki Yamamoto, all of Kitakyushu, Japan

[73] Assignee: Nippon Steel Corporation, Tokyo, Japan

[22] Filed: Sept. 24, 1971

[21] Appl. No.: 183,686

**Related U.S. Application Data**

[63] Continuation-in-part of Ser. No. 812,147, April 1, 1969, abandoned.

[30] **Foreign Application Priority Data**

Apr. 24, 1968 Japan..... 43-21686

[52] **U.S. Cl.** ..... 148/111, 75/123 L, 148/31.55, 148/112

[51] **Int. Cl.** ..... H01f 1/04

[58] **Field of Search** ..... 148/111, 31.55, 112, 110; 75/57, 123 L

[56] **References Cited**

**UNITED STATES PATENTS**

|           |         |                |       |         |
|-----------|---------|----------------|-------|---------|
| 2,913,361 | 11/1959 | Fitz           | ..... | 148/110 |
| 3,157,538 | 11/1964 | Imai et al.    | ..... | 148/110 |
| 3,159,511 | 12/1964 | Taguchi et al. | ..... | 148/111 |
| 3,287,183 | 11/1966 | Taguchi et al. | ..... | 148/111 |
| 3,333,993 | 8/1967  | Kohler         | ..... | 148/111 |

|           |         |                |       |         |
|-----------|---------|----------------|-------|---------|
| 3,540,948 | 11/1970 | Benford et al. | ..... | 148/112 |
| 3,671,337 | 6/1972  | Kumai et al.   | ..... | 148/111 |
| 3,700,506 | 10/1972 | Tanaka et al.  | ..... | 148/112 |

**OTHER PUBLICATIONS**

Baeyertz, M.; Nonmetallic Inclusions in Steel; Cleveland, (ASM) 1947, pp. 72-73.

Lyman, T.; Metals Handbook; Cleveland, Ohio, (ASM) 1948, pp. 450-451.

*Primary Examiner*—Walter R. Satterfield  
*Attorney, Agent, or Firm*—Wenderoth, Lind & Ponack

[57]

**ABSTRACT**

Ingot steel for use in producing a single-oriented silicon steel sheet having a high magnetic induction, the steel being a silicon steel containing less than 0.085% C, 1-3.5% Si, up to 0.060% S, 0.02 to 0.945% acid-soluble Al and at least one element selected from the group consisting of 0.007 to 0.30% Se, 0.077 to 0.20% Te and the rest being Fe. The ingot steel is hot-rolled to form a steel sheet, the hot-rolled steel sheet is subjected to an annealing for precipitating AlN in a temperature range of 850° to 1,200°C when Si is present in an amount of from 1 to 2.5%, and at a temperature range of 960° to 1,200°C when Si is present in an amount of 2.5 to 4%, the annealing being for a time of 30 seconds to 30 minutes. The annealed sheet is cold-rolled to obtain a steel sheet of final thickness, the cold-rolling being at a reduction rate of 60 to 95% when there is a single cold-rolling step, and when there is a plurality of cold-rolling steps the final cold-rolling step is at a reduction rate of 60 to 95%. The final steel sheet has a  $B_{10}$  value of over 19,100 gauss.

2 Claims, 2 Drawing Figures

PATENTED DEC 10 1974

3,853,641

SHEET 1 OF 2

FIG. 1



INVENTORS

Akira  
Satoru  
Toshiya  
Kiyoshi  
Takaaki

Sakakura  
Taguchi  
Wada  
Ueno  
Yamamoto

BY, *Wenderoth, Lind & Ponack*

ATTORNEYS

PATENTED DEC 10 1974

3,853,641

SHEET 2 OF 2

FIG. 2



INVENTORS

Akira  
Satoru  
Toshiya  
Kiyoshi  
Takaaki

Sakakura  
Taguchi  
Wada  
Ueno  
Yamamoto

BY, *Wenderoth, Lind & Ponack*

ATTORNEYS

## METHOD FOR PRODUCING SINGLE-ORIENTED SILICON STEEL SHEETS HAVING HIGH MAGNETIC INDUCTION

This application is a continuation-in-part of application Ser. No. 812,147, filed Apr. 1, 1969, now abandoned.

This invention relates to ingot steel and a method for producing from said ingot steel, single-oriented electromagnetic steel sheets having an easy magnetization axis <100> in the rolling direction of the steel sheet.

Single-oriented steel sheets are used mostly as iron cores for transformers and other electric devices. Therefore their magnetic characteristics, excitation characteristics and core loss values must be favorable.

Recently, it has become an important problem to make the size of electric devices such as transformers small and for this purpose a reduction in the weight of the core is required. In general, in order to be able to reduce the weight of the core to be used for electric devices a portion of a steel sheet, wherein the magnetic induction is high, must be used. Thus, a steel sheet having favorable magnetization characteristics, that is, a steel sheet having high  $B_{10}$  characteristics, is needed, and more particularly a greater importance is attached to a steel sheet having a high saturated magnetic induction  $B_s$ . Further, it should be understood that when using that portion of a steel sheet, wherein the magnetic induction is high, the core loss value generally increases. However, as compared with a material having low  $B_{10}$  characteristics, a steel sheet having high  $B_{10}$  characteristics has a much lower core loss in the region of high magnetic induction, and moreover the increase in the core loss is at a lower rate, as the magnetic induction rises.

Putting all points above-mentioned together, it can be said that an improvement in designed magnetic flux density which is to be unavoidably expected as the capacity of electric devices increases, can first be realized by providing electromagnetic steel sheets having very high magnetic induction.

The present invention has for its object the supply of products which can meet the requirements as above-mentioned. That is, according to the present invention it is possible to produce electromagnetic steel sheets which are markedly superior to any conventional single-oriented silicon steel sheets with respect to the magnetic induction  $B_{10}$  in the rolling direction, that is, steel sheets which have a magnetic induction above 19,100 gauss, and up to 20,100 gauss.

Heretofore, in conventional silicon steel sheets, the reduction in resistance and the deterioration of core loss values were due to the low content of Si. Apart therefrom, it was also not possible to obtain on an industrial scale steel sheets having crystals with a so-called  $\{110\} <100>$ -orientation. Consequently single-oriented steel sheets could not be obtained at all and their high  $B_s$  value could not be utilized. By the method of the present invention, there can be manufactured on an industrial scale ideal single-oriented electromagnetic steel sheets having high magnetic induction, that is, high  $B_{10}$  value, and moreover having a high  $B_s$  value, even when the Si content is low, by producing secondary recrystallization grains having very well selected  $\{110\} <100>$ -orientation, extending over a wide range of silicon content such as from 0 to 3.5%.

An object of the present invention is to provide a composition of ingot steel suited to the production of single-oriented silicon steel sheets having high magnetic induction.

5 Another object of the present invention is to provide a method for producing from said ingot steel single-oriented silicon steel sheets having high magnetic induction.

Other objects of the present invention will be made 10 clear by the following explanation and attached drawing.

FIG. 1 shows excitation characteristics of a typical product of the present invention and

15 FIG. 2 shows core loss values of the product of the present invention respectively.

The present invention relates to a method for producing single-oriented silicon steel sheets having high magnetic induction, in which a normal steel material or silicon steel material which contains C and Al as indispensable elements. In addition thereto, a small amount of either Se or Te or both and/or S are added to the above-mentioned steel materials according to known steel-making methods, melting methods and casting methods used in normal industrial techniques. The thus-prepared steel material is hot-rolled and then subjected to an annealing process and cold-rolling process one time or more respectively to make the final gauge. The thus obtained product is decarburized and then subjected to a final annealing to generate secondary recrystallization grains having  $\{110\} <100>$ -orientation in the steel material. The present invention is particularly characterized in that the final cold-rolling is carried out at a reduction rate of 60 to 95%, depending upon the Si content and one of the intermediate annealings after the hot-rolling or between a cold-rolling and a sequential cold-rolling step is carried out in such a temperature range that the  $\gamma$ -transformation may occur at least in a part of the steel material. This temperature range is 850° to 1,200°C. according to the Si content (hereinafter the said intermediate annealing is called a "special intermediate annealing"). These steps cause AlN of desirable size to precipitate, so that the magnetic induction in the rolling direction will reach above 19,100 gauss and maximum of 20,100 gausses.

40 The details of the present invention shall be explained in the following.

45 The normal steel or silicon steel material starting material in the present invention is an ingot made by solidifying, by any casting method, a molten steel made by a steel-making method which is already known, such as, for example, by an open-hearth furnace, an electric furnace or a converter or melted by such a known melting method as, for example, by a high frequency electric furnace or vacuum melting furnace. A slab-like ingot obtained by a continuous casting method, which recently came into wide use, can also be used as a material in the present invention. The atmosphere in the case of casting is usually air but may be a vacuum or an inert gas as well.

50 As described above, the material in the present invention may be made by any steel-making, melting and casting methods. But the composition of the material must satisfy the following conditions, irrespective of the methods for producing the same, that is, irrespective of what steel-making, melting and casting methods are used.

The material must contain less than 0.085% C, from 1-3.5% Si, and when Si is present, and 0.02 to 0.045% Al (however, Al means an acid-soluble Al, which will be hereinafter simply shown by Al). In addition thereto, either Se or Te or both are to be added as indispensable elements in the following ranges:

|    |                 |
|----|-----------------|
| Se | 0.007 to 0.300% |
| Te | 0.007 to 0.200% |

Further, in the present invention, the abovementioned composition can contain 0.003 to 0.060% S. It is necessary that C in the above-mentioned material should be present in an amount sufficient to produce a  $\gamma$ -transformation at least in a part of the steel in response to the Si content. According to our experiences, C in a steel ingot must be at least 0.025% where Si is 3% but may be about 0.005% where Si is 0%. In regard to the added elements, the inventors have the following view. Generally, in the production of a single-oriented electromagnetic steel sheet, a selected direction will be obtained since a secondary recrystallization in the  $\{110\} <100>$  direction occurs in the final annealing. However, in such case, the precipitate produced by the slight amount of added element, plays an important role. Such precipitate may be exemplified by nitrides, sulfides and oxides. Such role has been considered to merely finely disperse and precipitate the precipitate so that the normal grain growth will be inhibited and the secondary recrystallization will be accelerated. However, the present inventors have discovered that, besides the above-mentioned role of the precipitate, a part of the precipitate which has been precipitated in

strictly regulated direction in coexistence with AlN, whereby a stabilized process for industrially producing single-oriented electromagnetic steel sheets having a high magnetic induction ought to be able to be carried out. However, as a practical matter, if secondary recrystall grains accurately arranged in one direction are to be obtained, the allowable ranges of the composition and treating conditions will become so narrow that industrial stability must be sacrificed.

10 The present inventors have disclosed in U.S. Pat. No. 3,287,183 that, when 0.005 to 0.050% S is added, a single-oriented silicon steel sheet having a high magnetic induction stabilized by the coexistence of the AlN and sulfide can be produced and have further confirmed that Se and Te have the same effect as S. The utilization of Se and Te in a silicon steel is disclosed in U.S. Pat. No. 3,157,538 and others and the utilization of S is disclosed in U.S. Pat. No. 2,913,361. However, with only these silicon steels, the  $B_{10}$  characteristic of the product is less than 18,500 gauss and no single-oriented silicon steel sheet having such a high magnetic induction as the present invention can be obtained. The effects of Se and Te shall be described. Table 1 shows the relationship between the magnetic induction  $B_{10}$  and the elements S and Se of products obtained by hot-rolling each of 18 silicon steel ingots (made in an electric furnace) containing about 38% Si and about 0.029% Al so as to obtain a hot-rolled sheet of a thickness of 3 mm., first cold-rolling it at a reduction rate of 30%, then annealing it at 1,100°C. for 5 minutes, then finally cold-rolling it at a reduction rate of 85.7% so as to reach a final gauge of 0.30 mm., decarburizing it at 800°C. and finally box-annealing it at 1,200°C.

Table 1

| S<br>(wt.%)             | Secondary recrystall grain generation (generating rate in%) and $B_{10}$ characteristic (at a generating rate of 100%) |             |             |       |
|-------------------------|------------------------------------------------------------------------------------------------------------------------|-------------|-------------|-------|
|                         | no addition<br>(<0.003)                                                                                                | 0.028-0.033 | 0.075-0.086 | 0.120 |
| Se<br>(wt.%)            |                                                                                                                        |             |             |       |
| no addition<br>(<0.003) | 60%                                                                                                                    | 19,120      | 40%         | 10%   |
| 0.008                   | 18,510                                                                                                                 |             |             |       |
| 0.034                   | 18,990                                                                                                                 | 19,330      | 19,010      |       |
| 0.059                   |                                                                                                                        | 19,240      |             | 20%   |
| 0.093                   | 19,410                                                                                                                 |             |             |       |
| 0.157                   |                                                                                                                        | 19,350      | 18,750      | 10%   |
| 0.220                   | 19,140                                                                                                                 |             | 18,550      |       |
| 0.310                   | 20%                                                                                                                    |             |             | 0%    |

a specific directional relation with the matrix, further has the capacity for selectively growing only crystal grains in a specific direction, which strictly regulates the direction of the secondary recrystallized grains so that, as a result, a product with excellent  $B_{10}$  characteristics can be obtained. It has been confirmed that Al-nitride is very effective as a precipitate having such special action. Therefore, the formation of AlN forms the basis of the present invention. On the other hand, any nitrides other than AlN, as well as sulfides, oxides and other precipitates contribute to the secondary recrystallization in the sense of inhibiting the normal grain growth as described above but can not themselves regulate the secondary recrystallizing direction. Therefore, by the formation of only these precipitates, a product having such a high  $B_{10}$  characteristic as in the present invention can not be obtained, but they act for stably producing secondary recrystall grains in a very

55 As evident from this table, wherein the  $B_{10}$  characteristic values achieved according to the invention are outlined by a heavy line, in the case of no addition of S (S<0.003%), by adding about 0.090 to 0.300% Se in coexistence with AlN and with S up to about 0.033%, there can be obtained a product having a  $B_{10}$  characteristic of more than 19,100 gauss. Further, where S, Se and AlN coexist and when S is about 0.030%, most of the highest  $B_{10}$  characteristics can be obtained. That is to say, when there is no addition of Se (Se < 0.003%), S has been limited so as to be in the range of 0.005 to 0.050% (see U.S. Pat. No. 3,287,183). However, it has been found that, where AlN, S and Se coexist as in the present invention, by using 0.007 to 0.300% Se, the object of the present invention can be obtained, even though S is contained in a wider range of 0.003 to 0.060%. Further, when S is present only as an impurity, i.e., less than 0.003%, for a relatively high Si content in

the order of 3%, Se in the range of about 0.090 to about 0.30% will give high  $B_{10}$  characteristics.

Further, in regard to the Al content, the following fact has been found. Table 2 shows the relationship between the magnetic induction  $B_{10}$  and Se and Al in a final product made in exactly the same manner as in the treatment in Table 1 by hot-rolling each of 12 silicon steel ingots (made with an electric furnace) containing about 3% Si and about 0.030% S to a hot-rolled sheet of a thickness of 3 mm. The  $B_{10}$  values achieved according to the invention are outlined by a heavy line.

Table 2

| Al<br>(wt.%)            | Secondary recrystallization grain generation (generating rate in %) and $B_{10}$ characteristic (at a generating rate of 100%) |        |        |       |
|-------------------------|--------------------------------------------------------------------------------------------------------------------------------|--------|--------|-------|
| Se<br>(wt.%)            | 0.005                                                                                                                          | 0.015  | 0.031  | 0.080 |
| no addition<br>(<0.003) | 0%                                                                                                                             | 18,100 | 19,150 | 0%    |
| 0.030                   | 17,200                                                                                                                         | 18,600 | 19,180 | 40%   |
| 0.101                   | 17,600                                                                                                                         | 19,100 | 19,120 | 10%   |

It is found from this that, when Se is added, even for an Al content lower than in the case when only S is added, a product having a high  $B_{10}$  characteristic will be obtained.

Table 3

| S<br>(wt.%)             | Secondary recrystallization grain generation (generating rate in %) and $B_{10}$ characteristic (at a generating rate of 100%) |        |        |       |
|-------------------------|--------------------------------------------------------------------------------------------------------------------------------|--------|--------|-------|
| Se<br>(wt.%)            | no addition<br>(<0.003)                                                                                                        | 0.025  | 0.060  | 0.102 |
| no addition<br>(<0.003) | 20%                                                                                                                            |        | 40%    | 0%    |
| 0.007                   |                                                                                                                                | 19,980 |        |       |
| 0.030                   | 20,070                                                                                                                         | 19,850 | 19,760 | 20%   |
| 0.081                   | 19,730                                                                                                                         | 19,980 |        |       |
| 0.142                   | 19,320                                                                                                                         |        | 19,430 | 30%   |
| 0.230                   | 19,560                                                                                                                         |        |        | 10%   |
| 0.330                   |                                                                                                                                | 50%    | 30%    |       |

However, when the Al content is less than 0.010%, even if the secondary recrystallization is perfect, the  $B_{10}$  characteristic will be low and, when it is more than 0.045%, the secondary crystallization will be imperfect. In either case, the object of the present invention cannot be achieved.

Table 3 shows the relationship between the magnetic induction  $B_{10}$  and S and Se of a product obtained by hot-rolling each of 17 silicon steel ingots (made with an electric furnace).  $B_{10}$  values achieved according to the invention are outlined with a heavy line. The steel contains about 1% Si and, about 0.035% Al so as to be 2.0 mm. thick, and after hot-rolling, is continuously annealed in  $N_2$  at 1,050°C. for 2 minutes, then cold-rolled once at a reduction rate of 82.5% so as to reach a final gauge of a thickness of 0.35 mm., then decarburized (continuously annealing) at 800°C. and finally annealed in  $H_2$  at 950°C. for 10 hours.

From the results of many experiments including these results, the present inventors have reached the following conclusion. That is to say, when using a low Si material having less than 2.5% Si, even by the precipitation of only AlN, there will be obtained a product having a  $B_{10}$  characteristic of more than 18,500 gauss. However, when less than 0.300% Se is added thereto or

less than 0.60% S is further simultaneously added thereto, there will be obtained a particularly excellent single-oriented electromagnetic steel sheet having a high magnetic induction. This has been found to give the same effect as when using a high Si material having 2.5 to 3.5 Si. Further, the Al content in the steel ingot required to precipitate desirable AlN is 0.02 to 0.045%.

It has also been found that Te in a range of 0.007 to 0.200% has the same effect as Se. As shown by the examples, there has been obtained a product having a  $B_{10}$  characteristic exceeding 19,100 gauss by having AlN coexist with Te (0.007 to 0.200%), AlN coexist with Se (0.007 to 0.300%) and Te (0.007 to 0.200%), AlN coexist with S (0.003 to 0.060%), Se (0.007 to 0.300%) and Te (0.007 to 0.200%) or AlN coexist with Te (0.007 to 0.200%) and S (0.003 to 0.60%).

In the above, the effects of the coexistence of the three elements S, Se and Te with AlN in the present invention has been described. As described above, the precipitate produced by the addition of these elements coexists with AlN and plays a role in inhibiting the normal grain growth and accelerating the secondary recrystallization in the final annealing. Therefore, even in the present invention, in a step before the final annealing such as, for example, in the intermediate annealing or hot-rolling step, or at the time of heating it, or at the time of elevating the temperature in the final annealing, these elements may be made to diffuse into the steel sheet so as to be contained in fixed amounts.

It is reported, for example, in U.S. Pat. Nos. 3,333,991, 3,333,992 and 3,333,993 that S and Se can be rather easily made to diffuse into steel sheets.

In the present invention, too, needless to say, those methods can be used.

C is adjusted so as to be present in an amount below 0.080% so that a  $\gamma$ -transformation will occur in at least a part of the steel sheet due to the Si content while carrying out a special intermediate annealing.

That is to say, the summary is as shown in the following:

For less than 1% Si, less than 0.080% C is used (a steel ingot of less than 0.085% C).

For 1 to 2.5% Si, 0.010 to 0.080% C is used (a steel ingot of 0.015 to 0.085% C).

For 2.5 to 3.5% Si, 0.020 to 0.080% C is employed (a steel ingot of 0.025 to 0.085% C).

The C in the steel ingot is 0.005% higher than before the special intermediate annealing, because the decarburizing which takes place in the ordinary hot-rolling is taken into consideration. Essentially the C content in the steel sheet is important in carrying out the special intermediate annealing.

In case the C content exceeds the upper limit of the above-mentioned specified range, the generation of secondary recrystallization grains will become imperfect. On the other hand, when the C content becomes high, even if secondary recrystallization grains are obtained, the sharpness of the secondary recrystallization texture becomes low and the product which is the object of the present invention can not be obtained.

Si is present in an amount less than 3.5%. The present invention has an object to improve the  $B_{10}$  characteristic and  $B_s$  characteristic. Therefore, the lower limit is not defined. But, as regards the upper limit, if Si is present in an amount greater than 3.5%, the industrial cold-

rolling to produce the very high  $B_{10}$  value becomes impossible.

The basis for generating secondary recrystall grains having a particularly excellent orientation of the present invention is the formation of AlN. Therefore, in the present invention, the presence of any nitride other than that of Al and the nitride-forming elements must be noted in relation to the formation of AlN. As described above, the presence of the nitride contributes to the secondary recrystallization in the sense of inhibiting the normal grain growth and the presence of the nitride-forming element is significant. However, this should be determined in relation to AlN. That is to say, it is necessary that Zr and Ti which are elements stronger than Al in their affinity for N should be added depending on the amount of N contained in the steel by taking into consideration that AlN can be precipitated in a specified amount after the annealing as described later. B, Ta, Nb, V, Cr, Mn, W and Mo are weaker than Al in their affinity for N and therefore may well be added in proper amounts already known in the production of single-oriented silicon steel sheets. The allowable maximum values of the amounts of these elements are shown to be 1% for V, Mn and Mo, 0.5% for W and 0.1% for B, Zr, Ti, Nb, Ta and Cr. However, these are all only examples. It is not a deviation from the idea of the present invention to add elements in order to produce precipitates for the acceleration of the secondary recrystallization within a range which does not obstruct formation of AlN.

A material which has a composition conforming to the above-mentioned composition is made into product sheet thickness by at least one cold-rolling step. In such case, it is one of the features of the present application that the annealing after the hot-rolling or at least one intermediate annealing between the cold-rolling is carried out in a high temperature range in which a  $\gamma$ -transformation will occur in a part of the steel sheet so that a desirable size of AlN may be precipitated. This annealing temperature is in the range of 750° to 1,200°C. in which a  $\gamma$ -transformation will occur in response to the Si content.

It may be summed up as follows:

750° to 1,200°C. for less than 1% Si.

850° to 1,200°C. for 1 to 2.5% Si.

960° to 1,200°C. for 2.5 to 3.5% Si.

The annealing time in this temperature range is 30 seconds to 30 minutes.

When this annealing exceeds 30 minutes, the growth of crystal grains will occur during the annealing and the development of the secondary recrystall grains in the final annealing will become imperfect. Further, this annealing may be a box-annealing but generally it is industrially advantageous to carry it out by a continuous annealing. With an annealing for less than 30 seconds, the sought for effect can not be obtained. The annealing atmosphere is related to the precipitation of AlN required for the secondary recrystallization as already described. Usually the steel ingot obtained from an open-hearth furnace contains, without any additions, more than 0.0040% N which is sufficient to precipitate the required AlN. Therefore, so long as no remarkable denitration occurs, the annealing atmosphere may be a reductive or neutral atmosphere such as, for example, of H<sub>2</sub>, Ar, a gaseous mixture thereof or air. However, if the ingot is obtained by vacuum melting or the like, there will be so little N that it will be necessary to

add nitrogen in the annealing. The method of adding nitrogen is not critical but, in the present invention, it is recommended that the annealing be carried out in a neutral or reductive gas containing at least 10% N<sub>2</sub> by volume. The above-mentioned special intermediate annealing may be carried out at any time during the period after the hot-rolling until the final cold-rolling, and the time is not critical so long as it is in this period.

In the present invention, the cold-rolling is carried out one or more times and the final cold-rolling step may be carried out at a reduction rate of 60 to 95%, depending on the Si content so that the higher the Si content, the higher the reduction rate may be. It is not necessary to have any specific reduction rate in any other cold-rolling step. This can be said to be due to the effect of the coexistence of AlN, Se, Te and S in the material.

Any other intermediate annealing than the above-mentioned special intermediate annealing at a specified high temperature may be carried out at a temperature and for a time which are sufficient to make the cold-rolled structure a primary recrystall structure and are not critical. In the present invention, the number of times the cold-rolling step is repeated may be determined by the thickness of the hot-rolled sheet and the specified final cold-rolling reduction rate.

For example, when making a product 0.35 mm. thick from a hot-rolled sheet of 1 to 2.5% Si, if the thickness of the hot-rolled sheet is 1.4 to 3.5 mm., it is possible to treat the sheet by one strong cold-rolling process, after the AlN-precipitating annealing has been applied to the hot-rolled sheet. However, if the thickness is 3.5 mm., the sheet is treated in two cold-rolling steps. Further, if the hot-rolled sheet is thicker, it can be cold-rolled more than three times. However, from the industrial technical viewpoint, the hot-rolled sheet is usually 1.5 to 7 mm. thick.

The steel sheet of a product sheet thickness after the final cold-rolling is then subjected to a decarburizing annealing. This annealing is to make the cold-rolled structure a primary recrystall structure and at the same time to remove C which is detrimental when developing secondary recrystall grains in the {110}<100> direction in the final annealing. Any known process may be used for this step.

The final annealing should be carried out at such a temperature and for such a time that secondary recrystal grains in the {110}<100> direction can develop well. It is preferable to develop the secondary recrystal grains in a temperature range wherein no  $\gamma$ -transformation is produced in response to the Si content and at a temperature as high as industrially possible, because the generation of  $\gamma$ -transformation will change the once obtained secondary recrystal grains in the {110}<100> direction so that they are in another direction. When Si is present in an amount less than 1%, it should be carried out at 950°C. or usually at a temperature lower than that. However, the higher the Si content, the higher the temperature can be elevated.

When Si is present in an amount more than 2%, a temperature higher than 1,000°C. is possible. On the other hand, below 800°C., no secondary recrystallization will occur. Unless the temperature is made high, a product which has an excellent iron loss value can not be obtained. Therefore, with a low Si content, the  $B_{10}$  characteristic is excellent but the iron loss is worse than with a high Si content. The annealing time is sufficient

for the generation of secondary recrystallization grains if it is more than 1 hour but more than 5 hours is necessary in order to obtain a product having a low iron loss value with a high Si content. Further, no matter, whether the atmosphere is neutral, reductive or so weakly oxidative that the steel sheet will not be greatly oxidized, a product having a  $B_{10}$  characteristic of more than 19,100 gauss according to the present invention can be obtained. However, in order to obtain a low iron loss value with a high Si content, it is preferable to carry out the annealing in  $H_2$ . However, the description of such time and atmosphere has nothing to do with the substance of the present invention.

After Se, Te and S contained in the steel sheet have served for the development of secondary recrystallization grains in the  $\{110\} <001>$  direction in the finishing annealing by their coexistence with AlN, they are so detrimental to the magnetic property or particularly to the iron loss that it is necessary to remove them or reduce the amount thereof as much as possible. It is known to improve the free-cutting property by including Se or Te in a magnetic steel sheet product. However, the presence of such a large amount of Se or Te in the product is very disadvantageous to imparting required excellent magnetic characteristics to the product. Therefore, after it has served for the development of secondary recrystallization grains, it must be removed to a great a degree as possible. In order to remove Se, Te or S, the product may be annealed for a long time in  $H_2$ . Particularly, if more than 1.2% Si is present, Se, Te or S can be removed by annealing at a temperature of above 1,000°C. In order to attain the object of the present invention, it may be reduced to an amount less than 0.05%. Particularly, if it is reduced to an amount less than 0.01%, a favorable result can be obtained.

#### EXAMPLE 1

An Al-killed steel ingot containing 0.020% C, 0.041% Al, 0.024% S and 0.010% Se was bloomed and hot-rolled to a hot-rolled sheet 2.2 mm. thick. The content of C in the hot-rolled steel sheet was 0.017%. After this steel sheet was annealed in  $N_2$  at 950°C. for 2 minutes, it was pickled and cold-rolled to make the thickness of the sheet 0.50 mm. (at a reduction rate of 45 77.3%). Then, the cold-rolled steel sheet was decarburized by an open coil system at 750°C. for 5 hours.

The magnetic characteristics in the rolling direction of the product were as shown in FIG. 1(A), that is,

$$B_{10} = 19,950 \text{ gauss}$$

$$W_{15/50} = 3.60 \text{ watts/kg.}$$

#### EXAMPLE 2

A silicon steel ingot (prepared in an electric furnace) containing 0.030% C, 1.05% Si, 0.065% Se and 0.025% Al was bloomed and hot-rolled to a hot-rolled steel sheet 2.0 mm. thick. After this hot-rolled steel sheet was annealed in  $N_2$  at 950°C. for 2 minutes, it was pickled and cold-rolled to make the thickness of the sheet 0.50 mm. (at a reduction rate of 75%). Then, the cold-rolled steel sheet was decarburized by an open-coil system in a wet  $H_2$  at 750°C. for 5 hours and thereupon finally annealed in  $H_2$  at 950°C. for 10 hours. The product had magnetic characteristics in the rolling direction as shown in FIG. 1(B), that is,

$$B_{10} = 19,730 \text{ gauss}$$

$$W_{15/50} = 2.50 \text{ watts/kg.}$$

#### EXAMPLE 3

A silicon steel ingot containing 0.043% C, 2.15% Si, 0.010% S, 0.07% Se and 0.030% Al was bloomed and hot-rolled to a hot-rolled steel sheet 3.0 mm. thick. The C content of the hot-rolled steel sheet was 0.041% and was only slightly decarburized. This hot-rolled steel sheet was first cold-rolled by 30% to make the thickness of the sheet 2.1 mm. and then annealed in  $N_2$  at 1,100°C. for 2 minutes and thereafter pickled and cold-rolled to make the thickness of the sheet 0.35 mm. (at a reduction rate of 83.3%). The thus cold-rolled steel sheet was decarburized in a wet  $H_2$  at 800°C. for 3 minutes and then subjected to a final annealing, simultaneously attended with the desulfurization and deseleniumization. The magnetic characteristics in the rolling direction of the product were as shown in FIG. 1(C), that is,

$$B_{10} = 19,750 \text{ gauss}$$

$$W_{15/50} = 1.15 \text{ watts/kg.}$$

In the composition of the final product C was 0.005%, Se 0.005% and S 0.003%.

#### EXAMPLE 4

A silicon steel ingot containing 0.055% C, 2.95% Si, 0.025% S, 0.053% Se and 0.025% Al was bloomed and hot-rolled to a hot-rolled steel sheet 2.8 mm. thick. The C content of the hot-rolled steel sheet was 0.051%. The steel sheet was cold-rolled by 30% and then subjected to a continuous annealing in  $N_2$  at 1,150°C for 2 minutes. Then, the cold-rolled steel sheet was pickled and then again cold-rolled to make the thickness of the sheet 0.35 mm. (at a reduction rate of 82.1%). After the cold-rolled steel sheet was then decarburized in a wet  $H_2$  at 800°C. for 3 minutes, it was subjected to a final annealing at 1,200°C. for 20 hours, simultaneously attended with a desulfurization and deseleniumization.

The magnetic characteristics in the rolling direction of the product were as shown in FIG. 1(D), that is

$$B_{10} = 19,330 \text{ gauss}$$

$$W_{15/50} = 0.93 \text{ watts/kg.}$$

FIG. 2 shows the core loss of the product as an example. In the composition of the product C was 0.003%, S 0.002% and Se 0.003%.

#### EXAMPLE 5

A silicon steel ingot containing 0.075% C, 3.09% Si, 0.025% S, 0.030% Te and 0.060% Al was bloomed and hot-rolled to a hot-rolled steel sheet 3.2 mm thick. The C content of the hot-rolled steel sheet was 0.071%. The thus obtained hot-rolled steel sheet was first cold-rolled by 20% to a thickness of 2.56 mm. After the cold-rolled steel sheet was continuously annealed in  $N_2$  at 1,150°C. for 2 minutes, it was pickled and again cold-rolled to make the thickness of the steel sheet 0.30 mm. (at a reduction rate of 88.3%). Then, the thus cold-rolled steel sheet was decarburized in wet  $H_2$  at 850°C. for 2 minutes and then annealed at 1,200°C. for 20 hours. The magnetic characteristics in the rolling direction of the thus obtained product were as follows:

$$B_{10} = 19,120 \text{ Gausses}$$

$$W_{15/50} = 0.82 \text{ watts/kg.}$$

In the composition of the product C was 0.004%, S 0.003% and Te 0.008%.

## EXAMPLE 6

A silicon steel ingot containing 0.050% C, 3.12% Si, 0.041% Al, 0.030% S, 0.050% Se and 0.030% Te was hot-rolled to a hot-rolled steel sheet 3 mm. thick. After 5 the hot-rolled steel sheet was continuously annealed at 1,100°C. for 2 minutes, it was cold-rolled by 50%. Then, the cold-rolled steel sheet was annealed for a primary recrystallization at 900°C. for 1 minute and cold-rolled at a reduction rate of 84.7% to make the thickness of the sheet 0.23 mm. After the decarburization annealing, the steel sheet was subjected to a finishing annealing at 1,200°C. for 20 hours, simultaneously attended with a deselenization, detellurization and desulfurization. 15

The magnetic characteristics of the product were as follows:

$$B_{10} = 19,250 \text{ gauss}$$

$$W_{15/50} = 0.71 \text{ watts/kg.}$$

In the composition of the product C was 0.003%, S 20 0.003% and the sum of Se and Te 0.008%.

What is claimed is:

1. A process for producing a single-oriented silicon steel sheet having a magnetic induction value above 19,100 gauss consisting essentially of:

a. hot-rolling a silicon steel ingot consisting essentially of 0.015% to 0.085% C, 1-3.5% Si, with the proviso that when Si is present in an amount of

1-2.5%, C is present between 0.015% and 0.085% and when Si is present in an amount of 2.5-3.5%, C is present in an amount between 0.025% and 0.085%; S in an amount up to 0.060%, 0.02 to 0.045% acid soluble Al, and at least one element selected from the group consisting of 0.007 to 0.30% Se and 0.007 to 0.20% Te, more than about 0.004% N and the rest being Fe to produce a hot-rolled steel sheet;

b. annealing the hot-rolled steel sheet to precipitate AlN at a temperature range of 850° to 1,200°C when Si is present in an amount of from 1 to 2.5%, and at a temperature range of 960° to 1,200°C when Si is present in an amount of from 2.5 to 3.5%, the annealing being carried out for a time of 30 seconds to 30 minutes and

c. cold-rolling the thus-annealed steel sheet to obtain a steel sheet of final thickness, the cold-rolling being effected at a reduction rate of 60% to 95% when there is a single cold-rolling step and when there is a plurality of cold-rolling steps, the final cold-rolling step being carried out at a reduction rate of 60 to 95%.

2. The method claimed in claim 1 in which the silicon steel sheet contains 0.007 to 0.30% Se and 0.007 to 0.20% Te.

\* \* \* \* \*

30

35

40

45

50

55

60

65